

## UNITED STATES PATENT OFFICE

2,457,838

FLUORESCENT CELLULOSE ACETATE  
FILAMENTS

Richard R. Sitzler and George E. Dennison, Cumberland, Md., assignors to Celanese Corporation of America, a corporation of Delaware

No Drawing. Application May 4, 1946,  
Serial No. 667,499

2 Claims. (Cl. 8—50)

1

This invention relates to the preparation of colored fabrics, and relates more particularly to the production of fabrics woven of continuous or staple lengths of artificial filamentary materials such as, for example, regenerated cellulose, cellulose acetate, or other organic derivative of cellulose, dyed in shades which are extremely fast to light and which, in addition, exhibit a pronounced fluorescence under the excitation of ultra-violet light.

An object of this invention is the provision of colored fabrics made of or containing artificial filamentary materials which are dyed in shades fast to light and capable of fluorescence under the excitation of ultra-violet light in a color substantially identical with that of the fabric under visible light.

Another object of this invention is to provide colored fabrics of artificial filamentary materials containing fluorescent pigments and dyed in shades fast to light whereby the respective colorations produced will not interfere with each other, the fabric obtained being of the same color whether viewed by visible light or under ultra-violet light.

Other objects of this invention will appear from the following detailed description.

Artificial filaments or fibers which have been dyed with fluorescent dyestuffs so that they may glow under ultra-violet light have found some use in the arts. Thus, they may be employed in the manufacture of cloth for use in making uniforms and garments for show girls to produce spectacular stage effects. Also, they may be used in the manufacture of floor coverings in apartment buildings or in theatres, and the like, for indicating the presence of aisles, steps, etc. Usually, the fluorescent filaments or fibers are woven into the floor covering in a predetermined pattern. However, since the fluorescent dyestuffs may be entirely colorless when the ultra-violet source is withdrawn the pattern is no longer visible when illuminated by ordinary light. Furthermore, even when such portions of the floor covering which are also dyed with a dyestuff visible under ordinary illumination, as well as with a fluorescent dyestuff, are exposed to ultra-violet light so as to bring out the desired fluorescence, the ultra-violet light has an undesirable effect on the visible dyestuff, frequently causing fading, or even a complete change in shade on continued exposure, which shade may be undesirable. Fading is also produced in the case of fluorescent dyestuffs when the floor coverings containing filaments or fibers dyed with such dyestuffs are

2

subjected to continued exposure to sunlight as during daylight hours when the sunlight reaches the floor coverings through windows.

We have now found that artificial filamentary materials exhibiting the identical color under both daylight and the excitation of ultra-violet light may be obtained by incorporating a finely-divided fluorescent pigment in the spinning solution from which the artificial filaments are spun and then dyeing the filaments obtained in hank, bobbin or fabric form with a dyestuff highly resistant to changes in shade on continued exposure to ultra-violet light. The fluorescent pigment and the dyestuff to be employed therewith must be such that together they yield a color which does not vary appreciably when viewed by visible light or under ultra-violet light. Thus, various fabric materials may be formed wherein a decorative or identifying colored pattern is present in a color which is substantially identical regardless of whether the dyed materials are viewed by daylight or are illuminated by invisible, ultra-violet light.

The colored fluorescent filaments prepared in accordance with the process of our invention may have a basis of any suitable filament-forming material. The filaments may be formed by extruding a solution of the desired filament-forming material containing the desired finely-divided fluorescent pigment through a spinning jet containing a plurality of orifices into a medium adapted to effect the formation or solidification of the filaments. Thus, for example, the filaments may have a basis of regenerated cellulose which may be made by the viscose, cuprammonium, nitro cellulose, or any other process adapted for the production of said regenerated cellulose filaments. They may also have a basis of a synthetic linear polyamide condensation product or other suitable polymeric material such as polyvinyl chloride, polymerized vinylidene chloride, or a co-polymer of vinyl chloride and vinyl acetate.

Most advantageously, however, the improved filaments formed in accordance with our invention have a basis of an organic derivative of cellulose such as an organic acid ester of cellulose or a cellulose ether. Examples of organic acid esters of cellulose are cellulose acetate, cellulose propionate and cellulose butyrate, or mixed esters such as cellulose acetate-propionate and cellulose acetate-butyrate, while examples of cellulose ethers are ethyl cellulose and benzyl cellulose. The filaments having a basis of an organic derivative of cellulose may be prepared by dis-

solving the organic derivative of cellulose in a suitable volatile solvent, such as acetone, and extruding such solution, after the desired amount of finely-divided fluorescent pigment has been added thereto, through an orifice or plurality of orifices into an evaporative atmosphere as in the dry spinning method or into a liquid coagulating medium as in the wet spinning method, which spinning methods are well known in the art.

Prior to incorporation in the spinning solution, the fluorescent pigment is reduced to a very finely-divided form by a suitable treatment which may comprise grinding the pigment in a ball mill, colloid mill or the like, adapted to reduce the pigment to the desired finely-divided form. Preferably, the particles are reduced in size to a diameter of from less than 0.1 up to about 5 microns. The amount of pigment added will vary depending upon the particular shade which is desired in the filaments and the nature of the pigment employed. A satisfactory color of high intensity and brilliance under both daylight and ultra-violet light may be obtained by adding to the spinning solution an amount of fluorescent pigment of from about 0.01% to about 5 to 10% by weight, based on the amount of the filament-forming material present in the spinning solution.

The finely-divided colored fluorescent pigment may be added at any point in the manufacture of the filaments prior to extrusion. Thus, for example, a spinning solution may be prepared with the desired amount of fluorescent pigment incorporated therein and the pigmented spinning solution thus obtained then extruded through orifices to form filaments in the manner well known to the art. Most advantageously, however, the pigments may be added to the spinning dope at a point near the spinning jet or orifices through which it is extruded so that the system employed for spinning the filaments will not be contaminated with any particular color. This avoids extensive and time-consuming cleaning operations if it is desired to spin filaments in various other colors.

Because of the extremely fine particle size of the fluorescent pigments, the filaments obtained possess substantially the same tenacity and elongation characteristics as filaments which do not contain a finely-divided pigment. Consequently, the pigmented filaments prepared in accordance with my invention may be employed satisfactorily in any application where substantial tenacity and elongation characteristics are necessary.

As examples of fluorescent pigments which may be employed to impart the desired brilliant fluorescent color to the filaments, the following may be mentioned. For a yellow fluorescent color specially prepared mixtures of zinc sulfide and cadmium sulfide, or cadmium tungstate are satisfactory. For a red fluorescent color, specially prepared zinc sulfide, or mercuric oxide, potassium dichromate, magnesium dichromate, barium chromate, thorium dichromate, rhodium thiocyanate, as well as Rhodamine BX tungstate lake and Barium red lake C toner, are suitable. For a blue fluorescent color, we may employ pigments, such as specially prepared zinc sulfide of a blue fluorescent color, Peacock blue lake or certain blue dyestuffs in substance such as Milling Blue BC, Alizarine Blue SE. For a green fluorescent color, I have found that the addition of specially prepared zinc sulfide of a green daylight color as well as a green fluorescent color is suitable, as well as other pigments such as brilliant Green tungstate or Auramine 00 tungstate lake or Mala-

chite Green tungstate lake may be employed. A violet color may be obtained employing violet pigments such as ethyl violet tungstate lake. To obtain any other colors, the fluorescent pigments may be mixed as is well understood in the art.

The artificial filamentary materials containing the above finely-divided fluorescent pigments are then dyed with a suitable dyestuff resistant to the detrimental effects of ultra-violet light. The 10 filaments may be dyed in hank or in bobbin form or they may be woven in the desired fabric form and the fabric obtained then dyed in the piece. The dyestuffs preferably employed in dyeing pigmented cellulose acetate or other pigmented organic derivative of cellulose filaments comprise acid dyestuffs, such as those normally employed in the dyeing of wool, and those dyestuffs which are applied in dispersed form in the dyeing of cellulose acetate or other organic derivative of cellulose materials. Examples of said acid dyestuffs are Brilliant Sulfanine Red B, Artol Blue GL, Artol Yellow SG, Xylene Brilliant Cyanine G and Fast Red A, while examples of satisfactory dyestuffs applied in dispersed form are 1,4-di-25 methylaminoanthraquinone, the azo dyestuff obtained by coupling p-amino-acetanilide with p-cresol, and the azo dyestuff obtained by coupling p-nitro-aniline and dihydroxyethyl-m-toluidine. These dyes may also be incorporated in the 30 spinning solution in substance. When dyeing pigmented regenerated cellulose materials, dyestuffs such as Cotton Sky Blue FF, Amanil Fast Red 8BL (Color Index 278) or Chlorantine Yellow B (Color Index 814) may be employed. Surprisingly enough, the fastness of the dyeings on the 35 yarns containing fluorescent pigments is not affected by the fluorescent pigment present in the filaments being dyed.

Fluorescent pigmented yarns of high tenacity 40 may be obtained by subjecting those pigmented yarns having a basis of cellulose acetate, or other organic acid ester of cellulose, to a stretching operation whereby the filaments are stretched to 200, 300, 500 or even 1000, to 2000% of their original length. The yarns may be stretched to the desired degree when they are in a somewhat softened condition, which condition may be obtained by treating the fluorescent pigmented cellulose acetate yarns, or other organic ester of cellulose yarns, with organic solvents, latent solvents, or swelling agents therefor, or by subjecting the yarns to the action of hot water or steam at elevated temperature or pressure. The stretching of the yarns may be effected during, continuously with, or after their formation and the stretched yarns may then be taken up in suitable package form. The stretching operation causes cellulose acetate yarns to acquire a relatively high tenacity and this increased tenacity may be enhanced by subjecting the stretched cellulose acetate or other organic acid ester of cellulose yarns to saponification with a suitable alkaline medium.

The saponifying agent employed may be inorganic, such as, for example, sodium hydroxide, 65 potassium hydroxide, ammonium hydroxide or other organic basic agent, or may be an organic saponifying agent, such as, methyl amine, ethylene diamine, triethanolamine, or other organic base. The saponifying agents may be employed 70 in varying concentrations in aqueous, alcoholic or aqueous/alcoholic solutions and saponification may be effected satisfactorily at temperatures of 20 to 100°C.

The stretched cellulose acetate or other organic acid ester of cellulose yarns containing a

fluorescent pigment may be dyed after stretching with any of the dyestuffs heretofore mentioned or the stretched yarn may be dyed, after saponification, with suitable dyestuffs resistant to light and having an affinity for the regenerated cellulose material formed by saponification. The finely-divided fluorescent pigment contained therein does not affect the tenacity of the stretched and saponified yarns and they may be employed wherever such dyed, fluorescent yarns of high tenacity characteristics are desired.

In order further to illustrate our invention, but without being limited thereto, the following examples are given:

*Example I*

Cellulose acetate filaments containing a finely-divided fluorescent pigment are prepared by adding 1 part by weight of specially prepared zinc sulfide, fluorescent in a red color, to 400 parts by weight of a 25% solution of cellulose acetate in acetone and then extruding the mixture obtained through a spinning jet into an evaporative atmosphere where the volatile solvent is removed and the desired pigmented filaments are formed. The yarn obtained is then dyed in hank form by padding the hank of yarn with an aqueous dye-bath comprising 0.5 part by weight of p-nitro-benzene-azo-4-methyl-2-di-hydroxyethyl - amino-benzene on the weight of the yarn dispersed in 30 parts by weight of water, on the weight of the yarn, with the aid of sulfonated ricinoleic acid. Dyeing is effected at a temperature of 180° F. After being rinsed and dried, the yarn obtained is dyed in a bright red color and is fluorescent under ultra-violet light in a bright red color substantially identical with that under daylight. The yarn may also be dyed by padding the hank with 0.5 part by weight of Fast Red A (Color Index No. 176) on the weight of the yarn dispersed in 30 parts by weight of a 25% aqueous solution of ethyl alcohol containing 2% of sodium thiocyanate at 68° F. The yarn is dyed a bright color red and is fluorescent under ultra-violet light in a bright red color substantially identical with that under daylight.

*Example II*

Pigmented cellulose acetate filaments fluorescent in a yellow color are prepared by adding 1 part by weight of a mixture of specially prepared zinc sulfide and cadmium sulfide, fluorescent in a yellow color, to 400 parts by weight of a 25% solution of cellulose acetate in acetone and then extruding the mixture obtained through a spinneret as described in Example I to form the desired filaments. The yarns obtained are then dyed in hank form by padding the hanks with an aqueous dye-bath containing 0.5 part by weight of the azo dyestuff formed by coupling p-amino-acetanilide with p-cresol, the dye-bath being

maintained at 180° F. during dyeing. The hanks of yarn are rinsed and dried. The yarns are dyed a bright yellow shade and exhibit a bright yellow fluorescence under ultra-violet light. The 5 yarns may also be dyed a yellow color substantially identical with the yellow fluorescent color under ultra-violet light employing a dye-bath containing 0.5 part by weight of Artol Yellow SG on the weight of the yarn being dyed dissolved in 30 parts by weight of a 25% aqueous solution of ethyl alcohol containing 2% of sodium thiocyanate. The dyeing is carried out by padding with the dye-bath at 68° C.

It is to be understood that the foregoing detailed description is given merely by way of illustration and that many variations may be made therein without departing from the spirit of our invention.

Having described our invention, what we desire to secure by Letters Patent is:

1. In a process for the production of colored, fluorescent cellulose acetate filamentary materials exhibiting substantially the same color under visible as well as ultra-violet illumination, the step of dyeing the cellulose acetate textile material having incorporated therein a finely divided pigment consisting of zinc sulfide fluorescent in a red color with a dye-bath comprising p-nitro-benzene-azo-4-methyl-2-di-hydroxyethyl - amino-benzene, water and sulfonated ricinoleic acid.
2. Colored, fluorescent cellulose acetate filamentary materials exhibiting substantially the same color under visible as well as ultra-violet illumination having a finely divided pigment consisting of zinc sulfide fluorescent in a red color incorporated therein and colored with a fluorescent dyestuff consisting of p-nitro-benzene-azo-4-methyl-2-di-hydroxyethyl-amino-benzene.

RICHARD R. SITZLER.  
GEORGE E. DENNISON.

REFERENCES CITED

The following references are of record in the file of this patent:

UNITED STATES PATENTS

| Number    | Name         | Date          |
|-----------|--------------|---------------|
| 1,791,199 | Gardiner     | Feb. 3, 1931  |
| 1,875,894 | Singmaster   | Sept. 6, 1932 |
| 2,033,976 | Dreyfus      | Mar. 17, 1936 |
| 2,086,591 | Whitehead    | July 13, 1937 |
| 2,089,413 | Paine et al. | Aug. 10, 1937 |
| 2,142,717 | Dreyfus      | Jan. 3, 1939  |
| 2,169,657 | Millson      | Aug. 15, 1939 |
| 2,382,355 | Warren       | Aug. 14, 1945 |
| 2,412,817 | Lacey        | Dec. 17, 1946 |

FOREIGN PATENTS

| Number  | Country       | Date          |
|---------|---------------|---------------|
| 275,553 | Great Britain | May 25, 1928  |
| 348,094 | Great Britain | Oct. 31, 1929 |